

# United States Patent

[11] 3,546,369

[72] Inventors **Masami Ouki**  
Nagoya;  
**Masatoshi Suzuki, Okazaki-shi, Japan**  
[21] Appl. No. **3,342**  
[22] Filed **Jan. 16, 1970**  
Continuation-in-part of Ser. No. 730,305,  
May 20, 1968, abandoned  
[45] Patented **Dec. 8, 1970**  
[73] Assignee **Nippondenso Kabushiki Kaisha**  
**Kariya-shi, Aichi-ken, Japan**  
**a corporation of Japan**

2,635,975 4/1953 Pouzet..... 174/70(.1)UX  
2,645,819 7/1953 Peters..... 174/170(.1)UX

Primary Examiner—Laramie E. Askin  
Attorney—Cushman, Darby and Cushman

[54] **SPARK PLUG HAVING COMPOSITE INSULATOR**  
9 Claims, 4 Drawing Figs.

[52] U.S. Cl..... 174/152;  
161/188; 174/209; 313/137  
[51] Int. Cl..... H01t 13/38  
[50] Field of Search..... 174/152(S);  
209; 313/137; 161/188, 192, 193;  
65/43

[56] References Cited

UNITED STATES PATENTS

|           |        |                      |          |
|-----------|--------|----------------------|----------|
| 732,032   | 6/1903 | Barber.....          | 313/137  |
| 1,230,797 | 6/1917 | Schmidt .....        | 313/137  |
| 2,053,369 | 9/1936 | Jeffery.....         | 174/209X |
| 2,548,344 | 4/1951 | Buerger et al. ..... | 174/209X |

**ABSTRACT:** A spark plug having a composite insulator comprising a leg portion and a head portion formed of ceramic materials of different properties and compositions. In the insulator, the leg portion is formed of the first ceramic material consisting essentially of beryllium oxide which has a high heat conductivity and the head portion is formed of the second ceramic material consisting essentially of aluminum oxide which has a high mechanical strength, these portions being firmly chemically bonded to each other through at least one intermediate layer having a composition of 1—55 percent by weight of beryllium oxide, 30—89 percent by weight of aluminum oxide and 5—25 percent by weight of an additive, provided that, in the compositions of the respective layers, the sum of BeO and Al<sub>2</sub>O<sub>3</sub> is larger than 75 percent by weight and smaller than 95 percent by weight. The compositions change gradually from said first ceramic material to said second ceramic material. Said additive generally consists of at least one member selected from the group consisting of MgO, SiO<sub>2</sub>, CaO, BaO, TiO<sub>2</sub>, ZrO<sub>2</sub>, Fe<sub>2</sub>O<sub>3</sub>, NiO and MnO and preferably consists of about 5—25 percent by weight of two to three members selected from the group consisting of MgO, SiO<sub>2</sub> and CaO.



FIG. 1



FIG. 2



FIG. 4



INVENTORS

MASAMI OUKI  
MASATOSHI SUZUKI

BY

Cushman, Husley & Cushman  
ATTORNEYS

## SPARK PLUG HAVING COMPOSITE INSULATOR

## CROSS-REFERENCES TO RELATED APPLICATION

This is a Continuation-In-Part Application of U.S. application Ser. No. 730,305, filed on May 20, 1968, now abandoned.

## BACKGROUND OF THE INVENTION

## 1. Field of the Invention

This invention relates to the manufacture of a composite insulator having excellent thermal characteristics for spark plugs mounted on internal combustion engines for automotive vehicles, said insulator being divided into a leg portion consisting of a beryllia ceramic material having a high heat conductivity and a head portion consisting of an alumina ceramic material having high mechanical strength. These two portions are not connected with each other by any generally known cementation process or mechanical method, but are formed together as a unit with a gradually changing composition.

## 2. Description of the Prior Art

Previously known electrical insulators for spark plugs of this kind have been made of an alumina ceramic material consisting essentially of aluminum oxide and have a uniform composition throughout the insulator body. As is well known, the alumina ceramic material has a high mechanical strength, but the heat conductivity is relatively low compared with that of metals. Therefore, when such an insulator having a relatively large length of the leg portion is fitted in a spark plug, a large amount of heat is applied to the insulator and the temperature at the exposed end of the leg portion tends to increase, resulting in a tendency to give rise to preignition. On the other hand, an attempt to prevent undesirable preignition by shortening the length of the leg portion of the insulator results in a defect that the insulation is deteriorated by carbon and the like deposited during the running of the vehicles at a low speed. Especially, for mounting on a racing car engine a spark plug must have a satisfactory degree of heat dissipation, and for this purpose it has been common practice to employ an insulator having a length of its leg portion of about 3 to 4 millimeters. In the near future, the length of the leg portion will be further shortened and will possibly be reduced to zero in an extreme case. In such a case, the problem of insulation deterioration will become more outstanding.

In order to eliminate these vital defects, at present various kinds of insulators for spark plugs having varying lengths of the leg portion thereof are manufactured to suit various operating conditions. For this purpose, it has recently been proposed to make an electrical insulator for spark plugs of a ceramic material having an excellent heat conductivity. Among ceramic materials which may be used at high temperatures, a beryllia ceramic material consisting essentially of beryllium oxide has the highest heat conductivity. However, the beryllia ceramic material has a mechanical strength which is only about a half of that of the alumina ceramic material consisting essentially of aluminum oxide and is very expensive. The insulator for spark plugs must have a high mechanical strength at several parts thereof including the part projecting from the outer shell of the spark plug. Furthermore, the insulator occupies a greater part of the cost of a spark plug, and thus the cost of the insulator is also regarded as an important factor. Therefore, a filler material having a high mechanical strength such as aluminum oxide may be added to the beryllia ceramic material to improve the mechanical strength of the insulator and to reduce the cost of the insulator compared with an insulator for spark plugs made of beryllia ceramic material alone.

## SUMMARY OF THE INVENTION

The present invention which intends to overcome the above-mentioned defects is based on the idea that an improved insulator for spark plugs can be obtained by forming the leg portion of the insulator, where a high heat conductivity

is required, of a beryllia ceramic material consisting essentially of beryllium oxide, forming the head portion of the insulator, where a high mechanical strength is required of a ceramic material having an excellent mechanical strength and consisting essentially of aluminum oxide and bonding said leg portion of the insulator and said head portion of the insulator with a gradually changing composition by the use of a special ceramic material obtained by adding a small amount of an additive (oxide) to an appropriate mixture of the above-mentioned two ceramic materials.

It is therefore an object of the present invention to provide a composite insulator for spark plugs having a high heat conductivity and a high mechanical strength at a low cost. Another object of the invention is to adapt a certain kind of an insulator for spark plugs to a wider range of operating conditions. Still another object of the invention is to provide a composite insulator for spark plugs wherein the leg portion thereof is strongly bonded to the head portion thereof so that the insulator may be sufficiently strong to withstand a large bending force imparted thereto during assembly work. Still another object of the invention is to provide a spark plug which is most suitable for use in a high speed engine for racing cars.

In order to bond different ceramic materials, there has been known a method of mechanical bonding of those materials, a method involving the insertion of an appropriate refractory material between those materials and the mechanical bonding of the materials. A method for bonding different materials by a cementation process is also generally known. Also, it is known that a rubber and a synthetic resin can be chemically bonded by the use of a special technique due to the characteristics of the materials, and by particularly specifying an additive or an intermediate composition. Different ceramic materials have not heretofore been completely bonded with a gradually changing composition. We have now found that a beryllia ceramic material and a alumina ceramic material can be bonded with a gradually changing composition.

It is impossible to directly bond the ceramic material A consisting essentially of beryllium oxide with the ceramic material B consisting essentially of aluminum oxide which are used in the present invention. The material A and the material B should be equal in 1. thermal expansion coefficient, 2. melting point, 3. sintering velocity, 4. coefficient of contraction, 5. concentration gradient and 6. reaction product in order to strongly bond the materials with a gradually changing composition. Even if the material A is once bonded to the material B, the bonded insulator may be cracked and their bonding is not so simple.

According to the present invention, the material A and the material B are bonded by providing at least one intermediate layer between the two materials having intermediate characteristics with regard to 1. thermal expansion coefficient, 2. concentration gradient, 3. sintering velocity, etc. In the intermediate layer a mixing ratio of aluminum oxide and beryllium oxide, the number of such intermediate layers provided and the kind and amount of the additive used may be varied. In this case, the material A and the material B cannot be strongly bonded with a gradually changing composition if an intermediate layer consisting of a mere mixture of aluminum oxide and beryllium oxide is provided. A special composition must be developed in order to obtain an intermediate bonding material of desirable properties.

The present invention will be illustrated by the following examples in conjunction with the accompanying drawings.

## BRIEF DESCRIPTION OF THE DRAWING

FIG. 1 is a vertical section of a spark plug having composite insulator according to the present invention. FIG. 2 is a vertical section of a moulding apparatus employed for the manufacture of an insulator for spark plugs according to the present invention. FIG. 3 is a graphic illustration of the performance of a spark plug having an insulator according to the present invention compared with the performance of a spark plug hav-

ing a previously known insulator for spark plugs. FIG. 4 is a graphic illustration showing the relationship between the number of intermediate layers and the bending strength of the bonded insulator.

#### DESCRIPTION OF THE PREFERRED EMBODIMENT

Referring to FIG. 1, a composite insulator for spark plugs according to the present invention is composed of a leg portion 1a, a head portion 1b and an intermediate portion 1c connecting the leg portion 1a with the head portion 1b. The leg portion 1a is formed of a ceramic material consisting essentially of beryllium oxide which has a very high head conductivity, and the head portion 1b is formed of a ceramic material consisting essentially of aluminum oxide which has a high mechanical strength. The intermediate portion 1c is formed of a ceramic material having an intermediate composition between the compositions of said two ceramic materials. At the tip of an outer shell 2 of the spark plug there is formed a grounded electrode 4 opposite to a central electrode 3 which has been inserted into an axial bore in the leg portion of the insulator. The leg portion is shrunk onto the head portion of the insulator 1b by well known shrinkage means such as by electrical heating shrinkage. A rod for a high voltage terminal 5 is electrically connected with the central electrode 3. Numeral 6 is a sealing member. The structures of the outer shell 2, central electrode 3, grounded electrode 4, rod for high voltage terminal 5 and sealing member 6 are similar to those of previously known spark plugs.

The manufacture of a composite insulator 1 according to the present invention will be described with regard to a spark plug having the above-mentioned structure.

A moulding apparatus as shown in FIG. 2 was used for the manufacture of the composite insulator for spark plugs. The moulding apparatus comprised a cylindrical rubber mould 7 to which a moulding pressure was applied by the use of oil pressure from the outer periphery toward the center thereof. A core 9 had an integral needle 8 for forming an axial bore for receiving the central electrode and the rod for the high voltage terminal. A lower mould 10 provided a moulding cavity together with said cylindrical mould 7.

The ceramic materials having compositions A, B and C as shown in the following Table 1, which were necessary to form the desired composite insulator for spark plugs, were first prepared.

TABLE 1

| Component, percent by weight         | Composition           |                        |                        |
|--------------------------------------|-----------------------|------------------------|------------------------|
|                                      | A<br>First<br>ceramic | B<br>Inter-<br>mediate | C<br>Second<br>ceramic |
| BeO.....                             | 90-98                 | 10-30                  | .....                  |
| Al <sub>2</sub> O <sub>3</sub> ..... | 1-5                   | 55-85                  | 90-98                  |
| Additive.....                        | 1-9                   | 5-15                   | 2-10                   |

The composition A consisted essentially of beryllium oxide and the composition C consisted essentially of aluminum oxide. In case the intermediate layer comprises only one layer as shown in Table 1, the composition B for the intermediate layer consists of 10-30 percent by weight of BeO, 55-85 percent by weight of Al<sub>2</sub>O<sub>3</sub> and 5-15 percent by weight of an additive provided that the sum of BeO and Al<sub>2</sub>O<sub>3</sub> is larger than 85 percent by weight and smaller than 95 percent by weight. The additive may generally consist of at least one member selected from the group consisting of MgO, SiO<sub>2</sub>, CaO, BaO, TiO<sub>2</sub>, ZrO<sub>2</sub>, Fe<sub>2</sub>O<sub>3</sub>, NiO and MnO. It is desirable that said additive comprises 5 to 25 percent by weight of two to three members selected from the group consisting of MgO, SiO<sub>2</sub> and CaO.

A mass of a ceramic material 11 having the composition A was charged into the bottom portion of the moulding cavity

formed by the cylindrical rubber mould 7 and the lower mould 10 of the moulding apparatus as shown in FIG. 2. Ceramic material 12 having the composition B was then charged in a small amount. Finally, a ceramic material 13 having the composition C was charged as the uppermost layer. After completing the charging of these ceramic materials into the cylindrical rubber mould 7, a suitable moulding pressure of 200 to 1,000 kg/cm<sup>2</sup> was applied to the outer periphery of said cylindrical mould 7 to effect compression moulding. The moulded body was then subjected to cutting or grinding into the desired shape and fired at a suitable firing temperature of about 1600° C. During the firing step, the ceramic material 11 having the composition A reacted with the ceramic material 12 having the composition B at the bonded portion. A reaction product of chrysoberyl (BeO\*\*Al<sub>2</sub>O<sub>3</sub>) was partly formed and these ceramic materials were firmly bonded to each other. Thus, the leg portion of the insulator a formed of the beryllia ceramic material and the head portion of the insulator 1b formed of the alumina ceramic material were firmly bonded by the bonded portion 1c formed of the special ceramic material having an intermediate composition between the compositions of said ceramic materials to form a composite insulator for spark plugs 1 as shown in FIG. 1. As seen from FIG. 1, the bonded portion 1c did not show a distinct change in composition owing to the formation of said reaction product and a firm bonding was obtained possessing a gradually changing composition.

Such a composite insulator for spark plugs of such a structure shows high mechanical strength at the upper portion including the portion, where the outer shell of the spark plug is shrunk thereon, and the portion projecting from said outer shell —problems relating to mechanical strength. There is no problem relating to mechanical strength. Further, the leg portion of the composite insulator serving as a path of heat dissipation has a high heat conductivity and rapidly removes the large amount of heat which is generated at the portion to effectively prevent local overheating.

A spark plug as shown in FIG. 1 having the composite insulator for spark plugs according to the present invention and a spark plug having a prior art composite insulator for spark plugs formed of the known alumina ceramic material consisting essentially of aluminum oxide were compared with regard to the relationship between their preignition limits and the lengths of the leg portions of the insulators. Referring to FIG. 3, the preignition limit is taken as an ordinate and the length is millimeters of the leg portion of the insulator is taken as the abscissa. FIG. 3 shows that the relationship between the preignition limit and the length of the leg portion of the insulator is represented by a straight line E in the case of the former and by a straight line F in the case of the latter. At the same length of the leg portion of the insulator, the preignition limit of the former was about 1.5 times that of the latter. Also, at the same preignition limit, the length of the leg portion of the composite insulator of the former was about 2-3 mm. longer than that of the latter.

A spark plug having a composite insulator which has a selected length of the leg portion of the insulator according to the present invention may be advantageously used under both driving conditions in one of which a vehicle travels a long distance frequently running uphill or under a heavy load, and in the other of which a vehicle travels a short distance on a flat road in the city. Even under the former driving conditions in which the spark plug tends to be burnt, the very high heat conductivity of the leg portion of the insulator produces such a striking effect that a large amount of heat applied to the leg portion is quickly dissipated thereby to substantially eliminate any undesirable temperature increase at the lower end of the leg portion and to avoid preignition. Also, under the latter driving conditions in which the spark plug is liable to be fouled with carbon and other deposits the considerable length of the leg portion of the composite insulator produces such a remarkable effect that the lower end of the leg portion can be kept at a suitably low temperature thereby to avoid the deposi-

tion of carbon and the like materials at the leg portion and to eliminate undesirable deterioration of the insulation resistance. In other words, a single kind of spark plug may be adapted to a wide range of operating conditions.

The present invention is not limited to the specific embodiment illustrated above. The number of the intermediate layers may be also two, three, four and five. In each case, the compositions of the ceramic materials for forming each portion of the composite insulator spark plugs according to the present invention are limited as mentioned below.

In case of two intermediate layers, the compositions of the respective layers are shown in Table 2.

TABLE 2

| Component, percent by weight         | Composition   |             |              |                |
|--------------------------------------|---------------|-------------|--------------|----------------|
|                                      | First ceramic | First layer | Second layer | Second ceramic |
| BeO.....                             | 90-98         | 25-40       | 10-25        | .....          |
| Al <sub>2</sub> O <sub>3</sub> ..... | 1-5           | 45-70       | 55-80        | 90-98          |
| Additive.....                        | 1-9           | 5-15        | 10-20        | 2-10           |

The sum of BeO and Al<sub>2</sub>O<sub>3</sub> is larger than 80 percent by weight and smaller than 95 percent by weight. The additive is the same as in the case of one intermediate layer.

In case of three intermediate layers, the compositions of the respective layers are shown in Table 3.

TABLE 3

| Component, percent by wt.            | Composition   |             |              |             |                |
|--------------------------------------|---------------|-------------|--------------|-------------|----------------|
|                                      | First ceramic | First layer | Second layer | Third layer | Second ceramic |
| BeO.....                             | 90-98         | 30-45       | 15-30        | 5-15        | .....          |
| Al <sub>2</sub> O <sub>3</sub> ..... | 1-5           | 40-65       | 55-80        | 60-85       | 90-98          |
| Additive.....                        | 1-9           | 5-15        | 5-15         | 10-25       | 2-10           |

The sum of BeO and Al<sub>2</sub>O<sub>3</sub> is larger than 75 percent by weight and smaller than 95 percent by weight. The additive is the same as in the case of one intermediate layer.

In case of four intermediate layers, the compositions of the respective layers are shown in Table 4.

40

45

TABLE 4

| Component, percent by wt.            | Composition   |             |              |             |              |                |
|--------------------------------------|---------------|-------------|--------------|-------------|--------------|----------------|
|                                      | First ceramic | First layer | Second layer | Third layer | Fourth layer | Second ceramic |
| BeO.....                             | 90-98         | 35-50       | 20-35        | 10-20       | 3-10         | .....          |
| Al <sub>2</sub> O <sub>3</sub> ..... | 1-5           | 35-60       | 50-75        | 60-80       | 65-87        | 90-98          |
| Additive.....                        | 1-9           | 5-15        | 5-15         | 10-20       | 10-25        | 2-10           |

The sum of BeO and Al<sub>2</sub>O<sub>3</sub> is larger than 75 percent by weight and smaller than 95 percent by weight. The additive is the same as in the case of one intermediate layer.

In the case of five intermediate layers, the compositions of the respective layers are shown in Table 5.

65

TABLE 5

| Component, percent by wt.            | Composition   |             |              |             |              |             |                |
|--------------------------------------|---------------|-------------|--------------|-------------|--------------|-------------|----------------|
|                                      | First ceramic | First layer | Second layer | Third layer | Fourth layer | Fifth layer | Second ceramic |
| BeO.....                             | 90-98         | 40-55       | 25-40        | 15-25       | 5-15         | 1-5         | .....          |
| Al <sub>2</sub> O <sub>3</sub> ..... | 1-5           | 30-55       | 45-70        | 55-75       | 60-85        | 70-89       | 90-98          |
| Additive.....                        | 1-9           | 5-15        | 5-15         | 10-20       | 10-25        | 10-25       | 2-10           |

The sum of BeO and Al<sub>2</sub>O<sub>3</sub> is larger than 75 percent by weight and smaller than 95 percent by weight. The additive is the same as in the case of one intermediate layer.

As shown in FIG. 4, the bending strength of the bonded insulator varies according to the number of intermediate layers. If there is not present at least one intermediate layer, the electrical strength and mechanical strength of the spark plug will be insufficient for the spark plug to be put into practical use.

Regarding the respective points plotted on a curve showing the relationship between the bending strength of the bonded insulator and the number of intermediate layers in said FIG. 4, the representative examples of the compositions of the respective layers are shown as follows:

The first ceramic layer consists of 95.0 percent by weight of BeO, 1.0 percent by weight of Al<sub>2</sub>O<sub>3</sub> and 4.0 percent by weight of an additive. The second ceramic material consists of 95.0 percent by weight of Al<sub>2</sub>O<sub>3</sub> and 5.0 percent by weight of an additive. The compositions of intermediate layers are shown below for each number of the intermediate layers. The intermediate layers are successively numbered from the side closest to the first ceramic layer.

## (1) In the case of one intermediate layer:

| First layer                    |      |
|--------------------------------|------|
| Percent by wt.:                |      |
| BeO                            | 20.0 |
| Al <sub>2</sub> O <sub>3</sub> | 70.0 |
| MgO                            | 0.5  |
| SiO <sub>2</sub>               | 5.0  |
| CaO                            | 4.5  |

NOTE.—Bending strength of bonded insulator: 12.4 kg./mm.<sup>2</sup>

## (2) In the case of two intermediate layers:

|                                | First layer | Second layer |
|--------------------------------|-------------|--------------|
| Percent by wt.:                |             |              |
| BeO                            | 27.0        | 12.0         |
| Al <sub>2</sub> O <sub>3</sub> | 63.0        | 73.0         |
| MgO                            | 0.5         | 3.5          |
| SiO <sub>2</sub>               | 5.0         | 6.0          |
| CaO                            | 4.5         | 4.5          |

NOTE.—Bending strength of bonded insulator: 17.8 kg./mm.<sup>2</sup>

## (3) In the case of three intermediate layers:

|                                | First layer | Second layer | Third layer |
|--------------------------------|-------------|--------------|-------------|
| Percent by wt.:                |             |              |             |
| BeO                            | 30.0        | 18.0         | 6.1         |
| Al <sub>2</sub> O <sub>3</sub> | 60.0        | 72.0         | 74.2        |
| MgO                            | 0.5         | 0.5          | 9.7         |
| SiO <sub>2</sub>               | 5.0         | 5.0          | 5.0         |
| CaO                            | 4.5         | 4.5          | 5.0         |

NOTE.—Bending strength of bonded insulator: 20.1 kg./mm.<sup>2</sup>

## (4) In the case of four intermediate layers:

|                                | First layer | Second layer | Third layer | Fourth layer |
|--------------------------------|-------------|--------------|-------------|--------------|
| Percent by wt.:                |             |              |             |              |
| BeO                            | 37.0        | 22.0         | 12.0        | 5.0          |
| Al <sub>2</sub> O <sub>3</sub> | 53.0        | 68.0         | 70.5        | 75.0         |
| MgO                            | 1.0         | 1.0          | 8.0         | 10.0         |
| SiO <sub>2</sub>               | 4.5         | 4.5          | 6.0         | 5.0          |
| CaO                            | 4.5         | 4.5          | 4.5         | 5.0          |

NOTE.—Bending strength of bonded insulator: 19.9 kg./mm.<sup>2</sup>

## (5) In the case of five intermediate layers:

|                                | First layer | Second layer | Third layer | Fourth layer | Fifth layer |
|--------------------------------|-------------|--------------|-------------|--------------|-------------|
| Percent by wt.:                |             |              |             |              |             |
| BeO                            | 42.0        | 27.0         | 16.0        | 8.0          | 3.0         |
| Al <sub>2</sub> O <sub>3</sub> | 48.0        | 63.0         | 73.5        | 72.5         | 76.5        |
| MgO                            | 1.0         | 1.0          | 0.5         | 9.5          | 10.5        |
| SiO <sub>2</sub>               | 4.5         | 4.5          | 5.0         | 5.0          | 5.0         |
| CaO                            | 4.5         | 4.5          | 5.0         | 5.0          | 5.0         |

NOTE.—Bending strength of bonded insulator: 20.2 kg./mm.<sup>2</sup>

As described above, according to the present invention, the leg portion of a composite insulator is formed of a beryllia ceramic material consisting essentially of beryllium oxide, and the head portion of the composite insulator is formed of an alumina ceramic material consisting essentially of aluminum oxide. Thereby, a composite insulator for spark plugs of a high heat conductivity and a high mechanical strength may be provided which is excellent in heat conductivity at its portion requiring a high heat conductivity and it is also excellent in mechanical strength at the portion requiring a high mechanical strength. Furthermore, an effect that a spark plug can be used under a wide range of operating conditions is remarkable achieved because the leg portion of the composite insulator is formed of a beryllia ceramic material as described above. The composite insulator for spark plugs according to the present invention can be produced at a relatively low cost in spite of the fact that the leg portion is formed of an expensive beryllia ceramic material, because the leg portion occupies only about 75

one-third or less of the total volume of the insulator. As the leg portion and the head portion are bonded to each other through a ceramic material having a particular intermediate composition between the composition of the beryllia ceramic material and the composition of the alumina ceramic material, the bond between the leg portion and the head portion provided by a reaction between these ceramic materials at the bonded portion of the layers is a stronger than the bond obtained by merely bonding the leg portion to the head portion with glass or a heat resistant cement or by mechanical fabrication. The insulator can sufficiently withstand a strong bending force applied thereto during the assembly operation.

We claim:

1. A spark plug having a composite insulator comprising a leg portion consisting essentially of beryllium oxide and a head portion consisting essentially of aluminum oxide characterized in that said two portions are chemically bonded to each other through at least one intermediate layer consisting of 30 to 89 percent by weight of aluminum oxide, 1 to 55 percent by weight of beryllium oxide and 5 to 25 percent by weight of a ceramic oxide additive, provided that the sum of BeO and Al<sub>2</sub>O<sub>3</sub> is larger than 75 percent by weight and smaller than 95 percent by weight, and that the compositions of the respective intermediate layers gradually change from that of the head portion to that of the leg portion.
2. A spark plug according to claim 1, wherein the additive consists of at least one member selected from the group consisting of MgO, SiO<sub>2</sub>, CaO, BaO, TiO<sub>2</sub>, ZrO<sub>2</sub>, Fe<sub>2</sub>O<sub>3</sub>, NiO and MnO.
3. A spark plug according to claim 1, wherein the additive consists of about 5 to 25 percent by weight of two to three members selected from the group consisting of MgO, SiO<sub>2</sub> and CaO.
4. A spark plug according to claim 1, wherein the number of said intermediate layers is 3 to 5.
5. A spark plug according to claim 1, which on has one intermediate layer consisting of 10 to 30 percent by weight of BeO, 55 to 85 percent by weight of Al<sub>2</sub>O<sub>3</sub> and 5 to 15 percent by weight of the additive, provided that the sum of BeO and Al<sub>2</sub>O<sub>3</sub> is larger than 85 percent by weight and smaller than 95 percent by weight.
6. A spark plug according to claim 1, which has two intermediate layers, the composition of the first layer being 25 to 40 percent by weight of BeO, 45 to 70 percent by weight of Al<sub>2</sub>O<sub>3</sub> and 5 to 15 percent by weight of the additive and the composition of the second layer being 10 to 25 percent by weight of BeO and 55 to 80 percent by weight of Al<sub>2</sub>O<sub>3</sub> and 10 to 20 percent by weight of the additive, provided that the sum of BeO and Al<sub>2</sub>O<sub>3</sub> is larger than 80 percent by weight and smaller than 95 percent by weight.
7. A spark plug according to claim 1, which has three intermediate layers, the composition of the first layer being 30 to 45 percent by weight of BeO, 40 to 65 percent by weight of Al<sub>2</sub>O<sub>3</sub> and 5 to 15 percent by weight of the additive and the composition of the second layer being 15 to 30 percent by weight of BeO, 55 to 80 percent by weight of Al<sub>2</sub>O<sub>3</sub> and 5 to 15 percent by weight of the additive and the composition of the third layer being 5 to 15 percent by weight of BeO, 60 to 85 percent by weight of Al<sub>2</sub>O<sub>3</sub> and 10 to 25 percent by weight of the additive, provided that the sum of BeO and Al<sub>2</sub>O<sub>3</sub> is larger than 75 percent by weight and smaller than 95 percent by weight.
8. A spark plug according to claim 1, which has four intermediate layers, the composition of the first layer being 35 to 50 percent by weight of BeO, 35 to 60 percent by weight of Al<sub>2</sub>O<sub>3</sub> and 5 to 15 percent by weight of the additive, the composition of the second layer being 20 to 35 percent by weight of BeO, 50 to 75 percent by weight of Al<sub>2</sub>O<sub>3</sub> and 5 to 15 percent by weight of the additive, the composition of the third layer being 10 to 20 percent by weight of BeO, 60 to 80 percent by weight of Al<sub>2</sub>O<sub>3</sub> and 10 to 20 percent by weight of the additive and the composition of the fourth layer being 3 to 10 percent by weight of BeO, 65 to 87 percent by weight of Al<sub>2</sub>O<sub>3</sub> and 10 to 25 percent by weight of the additive, provided that

the sum of BeO and Al<sub>2</sub>O<sub>3</sub> is larger than 75 percent by weight and smaller than 95 percent by weight.

9. A spark plug according to claim 1, which has five intermediate layers, the composition of the first layer being 40 to 55 percent by weight of BeO, 30 to 55 percent by weight of Al<sub>2</sub>O<sub>3</sub> and 5 to 15 percent by weight of the additive, the composition of the second layer being 25 to 40 percent by weight of BeO, 45 to 70 percent by weight of Al<sub>2</sub>O<sub>3</sub> and 5 to 15 percent by weight of the additive, the composition of the third layer being 15 to 25 percent by weight of BeO, 55 to 75 per-

cent by weight of Al<sub>2</sub>O<sub>3</sub> and 10 to 20 percent by weight of the additive, the composition of the fourth layer being 5 to 15 percent by weight of BeO, 60 to 85 percent by weight of Al<sub>2</sub>O<sub>3</sub> and 10 to 25 percent by weight of the additive and the composition of the fifth layer being 1 to 5 percent by weight of BeO, 70 to 89 percent by weight of Al<sub>2</sub>O<sub>3</sub> and 10 to 25 percent by weight of the additive, provided that the sum of BeO and Al<sub>2</sub>O<sub>3</sub> is larger than 75 percent by weight and smaller than 95 percent by weight.